

# United States Patent Office

3,156,558

Patented Nov. 10, 1964

1

3,156,558

## HIGH-DENSITY, NONMAGNETIC STAINLESS STEEL

Samuel J. Rosenberg and Thomas P. Royston, Jr., Washington, D.C., assignors to the United States of America as represented by the Secretary of Commerce

No Drawing. Filed Oct. 3, 1961, Ser. No. 142,740

4 Claims. (Cl. 75—128)

This invention relates to a high density, nonmagnetic stainless steel.

By long established custom, the values of weights have been expressed as weight in air against standards having a density of 8.4 grams per cubic centimeter. Weights

5 out in air in a 16 pound laboratory induction furnace and the metal was poured into the form of 1½ inch diameter bars. These were given a four-hour homogenizing anneal in vacuum at 2000° F. prior to hot working. The steels

were hot worked by forging and swaging to rods of about 0.6 inch diameter. Hot working was carried out in the temperature range of about 2100 to 1600° F.

10 After hot working, the rods were cut into lengths of about 6 inches and turned between centers for cleaning. Samples of the clean, hot-worked material were then taken for spectrochemical and chemical analyses and for determination of density and magnetic permeability. The analyses of the two steels that closely approached the desired density are shown in the following table:

Table II

| National Bureau of Standards Mark | Percent |           |         |          |        |          |          |
|-----------------------------------|---------|-----------|---------|----------|--------|----------|----------|
|                                   | Carbon  | Manganese | Silicon | Chromium | Nickel | Tungsten | Nitrogen |
| SW-12                             | 0.09    | 1.7       | 1.55    | 16.2     | 32.4   | 9.9      | 0.017    |
| SW-13                             | 0.05    | 1.7       | 1.49    | 16.4     | 32.4   | 9.9      | 0.017    |

Determination of permeability and density gave the following values:

Table III

| National Bureau of Standards Mark | Magnetic Permeability (H=300 Oersteds) |             |                | Density, g. per cu. cm. |             |
|-----------------------------------|----------------------------------------|-------------|----------------|-------------------------|-------------|
|                                   | As Hot Worked                          | As Annealed | As Cold Worked | As Hot Worked           | As Annealed |
| SW-12                             | 1.008                                  | 1.019       | 1.03           | 8.42                    | 8.44        |
| SW-13                             | 1.009                                  | 1.024       | 1.03           | 8.45                    | 8.45        |

that have this density may be compared without a correction for air buoyancy being required.

Brass having a density of 8.4 g. per cu. cm. has been used for many years as material for standard weights. It is nonmagnetic, a necessary property for standards of mass. It is not, however, an ideal material since it tarnishes and thus is subject to changes in weight.

Accordingly, it is an object of the present invention to provide a stainless steel that has the required density and is nonmagnetic.

This is accomplished by increasing the density of an austenitic stainless steel by the addition of tungsten and maintaining austenite stability by proper balance of chromium and nickel. The preferred percent of elements and the range or maximum percent of elements, besides iron and the usual impurities, used in the present invention are indicated in the following composition table:

Table I

|            | Composition, percent |                  |
|------------|----------------------|------------------|
|            | Preferred            | Range or Maximum |
| Carbon     | 0.10                 | 0.20 max.        |
| Manganese  | 1.70                 | 2.00 max.        |
| Phosphorus |                      | 0.040 max.       |
| Sulfur     |                      | 0.030 max.       |
| Silicon    | 1.25                 | 1.60 max.        |
| Chromium   | 16.5                 | 15.5 to 17.5.    |
| Nickel     | 32.5                 | 31.5 to 33.5.    |
| Tungsten   | 9.5                  | 9.0 to 10.0.     |

In the execution of this invention, several experimental steels were melted and fabricated. Melting was carried

40 It is noted that an increase in magnetic permeability was obtained after annealing the hot-worked material. The remanent induction of the hot-worked specimens was measured after they had been subjected to magnetizing forces of several thousand oersteds. The measured remanent induction was negligible in comparison with the earth's field.

45 It is understood that while laboratory techniques were used in preparing the above alloys, which were given by way of example, other conventional furnace procedures may be followed in using the present invention.

50 What is claimed is:

1. A high density, nonmagnetic steel, of approximately 8.4 grams/cm.<sup>3</sup> and consisting essentially of:

55 carbon ..... 0.20% maximum  
manganese ..... 2.00% maximum  
phosphorous ..... 0.040% maximum  
sulfur ..... 0.030% maximum  
silicon ..... 1.60% maximum  
chromium ..... 15.5 to 17.5%  
nickel ..... 31.5 to 33.5%  
60 tungsten ..... 9.0 to 10.0%  
and the balance of said steel being essentially iron.

65 2. A high density, nonmagnetic steel of approximately 8.4 grams/cm.<sup>3</sup> and consisting essentially of:

65 carbon ..... 0.10%  
manganese ..... 1.70%  
silicon ..... 1.25%  
chromium ..... 16.5%  
nickel ..... 32.5%  
70 tungsten ..... 9.5%  
and the balance of said steel being essentially iron.

3. A high density, nonmagnetic steel of approximately 8.4 grams/cm.<sup>3</sup> and consisting essentially of:

|           |        |
|-----------|--------|
| carbon    | 0.09%  |
| manganese | 1.7%   |
| silicon   | 1.55%  |
| chromium  | 16.2%  |
| nickel    | 32.4%  |
| tungsten  | 9.9%   |
| nitrogen  | 0.017% |

and the balance of said steel being essentially iron.

4. A high density, nonmagnetic steel of approximately 8.4 grams/cm.<sup>3</sup> and consisting essentially of:

|           |       |
|-----------|-------|
| carbon    | 0.05% |
| manganese | 1.7%  |
| silicon   | 1.49% |
| chromium  | 16.4% |
| nickel    | 32.3% |

|          |        |
|----------|--------|
| tungsten | 9.9%   |
| nitrogen | 0.017% |

and the balance of said steel being essentially iron.

|           |          |               |
|-----------|----------|---------------|
| 1,528,478 | Hadfield | Mar. 3, 1925  |
| 1,542,233 | Girin    | June 16, 1925 |
| 1,953,229 | Heron    | Apr. 3, 1934  |
| 1,991,438 | Wohrman  | Feb. 19, 1935 |
| 2,587,613 | Payson   | Mar. 4, 1952  |

References Cited in the file of this patent  
UNITED STATES PATENTS

Evans: Wrought Heat Resisting Alloys for Gas Turbine Service, Reprint No. 31, reprinted from November 1945 issue of Metal Progress, page 4.

Gregg: Alloys of Iron and Tungsten, published for the Engineering Foundation by the McGraw-Hill Book Co., Inc., New York and London, 1934, pages 401 to 404.

#### OTHER REFERENCES